

H. H. HUGHES.

A. H. HUGHES.

METHOD OF TREATING ZINC ORES FOR THE RECOVERY OF METALLIC ZINC THEREFROM.

APPLICATION FILED APR. 6, 1910.

980,641.

Patented Jan. 3, 1911.

2 SHEETS—SHEET 1



Witnesses:

*Inventor.*

Jas. Hutchinson:  
Thos. R. Strath.

Harry H. Hughes,  
By F. R. Cornwell Attorney:

H. H. HUGHES,  
METHOD OF TREATING ZINC ORES FOR THE RECOVERY OF METALLIC ZINC THEREFROM,  
APPLICATION FILED APR. 6, 1910.

980,641.

Patented Jan. 3, 1911.

2 SHEETS—SHEET 2.

Fig. 2.



Fig. 3.



Fig. 4.



Witnesses:

Jas. S. Hutchinson:  
Thos. R. S. French.

By Harry H. Hughes,  
F. R. Cornwall Attorney

Inventor:

# UNITED STATES PATENT OFFICE.

HARRY H. HUGHES, OF SPRINGFIELD, MISSOURI, ASSIGNOR OF ONE-HALF TO F. X. HEER AND A. J. EISENMAYER, BOTH OF SPRINGFIELD, MISSOURI.

## METHOD OF TREATING ZINC ORES FOR THE RECOVERY OF METALLIC ZINC THEREFROM.

980,641.

Specification of Letters Patent. Patented Jan. 3, 1911.

Application filed April 6, 1910. Serial No. 553,770.

*To all whom it may concern:*

Be it known that I, HARRY HERBERT HUGHES, a citizen of the United States, residing at Springfield, in the county of 5 Greene and State of Missouri, have invented certain new and useful Improvements in Methods of Treating Zinc Ores for the Recovery of Metallic Zinc Therefrom, of which the following is a specification.

10 This invention relates to improvements in methods of treating zinc ores for the recovery of metallic zinc therefrom.

The object of the invention is the provision of a continuous method of treating 15 zinc ores in such a way that a greater quantity of ore may be efficiently treated within a given time to obtain a maximum amount of metal therefrom than with the methods heretofore employed.

20 A further object of the invention is the recovery of metallic zinc from its ores by the volatilization of the metallic zinc by a continuous method of treatment, the ores being continuously fed into a heated retort 25 where they are agitated, the volatile metal and residue being passed from said retort to a condenser, from which the condensed metal and residue are removed from time to time.

30 Other objects of the invention will be apparent from the detailed specification hereinafter when read in connection with the accompanying drawing wherein one form of apparatus is illustrated which may be used 35 to carry out the process and wherein like numerals of reference refer to similar parts in the several views.

In the accompanying drawings, Figure 1 40 is a longitudinal section of an apparatus which may be utilized in practicing the improved method, Fig. 2 is a vertical section taken on line 2—2 on Fig. 1, looking in the direction indicated by the arrow s, Fig. 3 is a vertical section on line 3—3 of Fig. 1. Fig. 4 is a vertical section on line 4—4 of Fig. 1.

45 For the purpose of illustration, I have shown in the accompanying drawings as one form of apparatus with which the improved method may be practiced, the apparatus disclosed in Patent No. 922906 issued the 25th day of May, 1909, to me for improvements in revolving furnaces for volatilizing ore, but it will of course be under-

stood that other forms of apparatus may be 55 utilized to carry on the improved method of treating zinc ores herein set forth.

In the apparatus shown 1 indicates the fire brick and walls and 2 the base of a supporting structure upon which rest the bearing brackets 37, supporting the revolving furnace which holds the retort 3. The retort 3, which is of tubular, and may be of gradually tapering form, is arranged with one end projecting through and beyond one 60 of the end walls, and terminates at its opposite end in a tubular feed extension 4, which projects through the other end wall and around which is secured a main hopper 26, which may be of any desired construction. 65 Positioned within the hopper 26 is a smaller or secondary hopper 27, from which a tube 28 extends into the feed extension 4 of the retort 3, which extension is provided on its inner surface with a feed screw which serves 70 to continuously feed ore from the hopper 27 into the retort during rotation thereof. In carrying out the method both hoppers are at all times kept full of ore thereby preventing the entrance of air into the retort, which is 75 absolutely necessary in distilling zinc ores for the recovery of metallic zinc. Surrounding and entirely inclosing the retort 3 is a cylindrical steel casing 5 provided with an inner lining 6 of fire brick, the retort 3 being 80 held in the proper relation by radial braces 7 extending between the same and the casing 5. The annular space 31 between the retort and the steel casing 5 provides a combustion chamber which is heated by oil or 85 gas burners 32 which extend through the front wall into said chamber. A flue or uptake in the front wall leads from said chamber. The steel casing 5 turns or rotates upon two pairs of bearing rollers 36 mounted 90 upon the upper ends of bearing brackets 37.

A hollow tube 8 has its inner end coupled or connected to the projecting end 9 of the retort 3 in any suitable manner and its opposite end extends through a stuffing box 10 100 arranged at the outer end of the upper hollowed portion 11 of an upright frame 12. The tube 8 constitutes a condensing chamber and the hollowed out portion of the frame 12 105 a continuation thereof. Mounted in the hollow frame 12 which constitutes a part of the condensing chamber, are two superposed slides 39 and 40, for a purpose to be herein-

after more particularly set forth, and leading from the hollow frame 12 just above the slide 39 is a duct 33 which permits the condensed metal to pass from the condensing chamber and to the collecting pan of a truck 34 or other suitable receptacle. The carbon monoxide gas which is generated by reducing the zinc ore passes from the condensing chamber into a pipe 35 by means of which it is led 5 into the combustion chamber 31 preferably at a point between the burner 32, and is used as an auxiliary fuel in maintaining the desired heat in said chamber. The condensing chamber may be made of the exact size and 10 kept at the exact temperature for the perfect condensation of the zinc fumes, thus reducing to a minimum the formation of "blue powder". In this connection it may be said that with the methods heretofore followed, 15 the formation of blue powder often amounts to as much as one half the zinc regularly discharged into the retort and that this powder has to be re-distilled only to be formed again and again. To insure maintaining the 20 proper temperature for the condenser, auxiliary gas heaters 42 may be used if necessary, and an auxiliary gas heater may also be arranged under the duct 33 to keep the zinc in a molten state. 25

30 In the form of apparatus herein illustrated, the tube 8 and retort 3 are rotated together by the following means. A motor 14 is arranged near the rear end wall, the shaft 15 of which is provided at one end with a pinion 16 which intermeshes with a large gear wheel 17 keyed or otherwise fixed to the rear end of a shaft 18 extending through the front end wall 1, and through a bearing 19 arranged beneath the center of the furnace and upon the supporting base 2. The gear 17 is also provided on one face with a pinion 20 which intermeshes with a second larger gear 21 keyed to the tube 8. The front or inner end of the shaft 18 is provided 35 with a pinion 22 which intermeshes with the gear 23 on the revolving furnace, it being understood that the pinions 20 and 22 respectively, and the gears 21 and 23, respectively, are of corresponding dimensions in 40 order that the furnace and the tube 8 will turn at exactly the same speed. The inner end of the tube 8 turns upon a pair of roller bearings 24 mounted at the upper end of a supporting bracket 25 bolted to the rear 45 end wall 1 of the supporting structure. 50

With the apparatus herein described, in carrying out the method, the hoppers 26 and 27 are filled with ore and the retort 3, which has previously been brought to the 55 proper temperature by the burners in the combustion chamber 31 is rotated, which

serves to draw ore therein from the hopper 27. The ore which is thus drawn into the retort is agitated by the rotation thereof and every particle of the ore is at once brought 65 into direct contact with the heat and carbon, so that the distillation of the metal contained therein is immediate and constant. The zinc vapors and the residue pass, during the rotation of the retort into the condensing chamber and a new supply of ore is continuously drawn into the retort from the hopper 27. After the zinc vapor which passes into the condenser has been condensed it passes off through the duct 33, which is so 70 formed as to prevent the entrance of any air to the retort. The residue is deposited on the slide 38 in the condensing chamber and when a sufficient amount has accumulated thereon this slide may be drawn out and the residue permitted to fall upon the lower slide 40 and by pulling out the latter slide after closing the former, the residue may be removed from the condensing chamber without admitting air to the retort. 75

I claim:—

1. The continuous method of volatilizing metallic zinc from its ores, consisting in introducing the ores into a heated retort, agitating the ores while contained within the 90 retort, passing the volatilized metal and residue from the retort into a condensing chamber, permitting the escape of the condensed metal from the condensing chamber, and removing the residue from the condensing 95 chamber.

2. The continuous method of volatilizing metallic zinc from its ores consisting in subjecting a body of ore to the action of heat, agitating the ore while being heated, passing 100 the volatilized metal into a condenser, applying heat to the condenser, allowing the condensed metal to escape from the condenser, and abstracting the combustible gases from the condenser. 105

3. The continuous method in volatilizing metallic zinc from its ores consisting in subjecting a moving body of ore to the action of heat to separate the volatile from the non-volatile portions thereof, condensing the volatile metallic vapors, and separating the condensed metal from the non-volatile residue, said heating, condensation and separation being effected without admitting air to the material under treatment. 110

In testimony whereof I affix my signature in presence of two witnesses.

HARRY H. HUGHES

Witnesses:

M. P. GILCHRIST  
W. M. BICKER